

# UNITED STATES PATENT OFFICE.

BURNELL R. TUNISON, OF NEW YORK, N. Y., ASSIGNOR TO U. S. INDUSTRIAL ALCOHOL CO., A CORPORATION OF WEST VIRGINIA.

## FUEL OF LIQUID TYPE.

1,423,049.

Specification of Letters Patent. Patented July 18, 1922.

No Drawing.

Application filed April 12, 1920. Serial No. 373,307.

To all whom it may concern:

Be it known that I, BURNELL R. TUNISON, a citizen of the United States, residing at New York, in the county of New York and State of New York, have invented a certain new and useful Improvement in Fuels of Liquid Type, of which the following is a specification.

My invention relates particularly to fuels 10 designed to be used in any desired manner. It has application especially to fuels adapted to be used alternatively for a wide variety of purposes, as for example, for burners under steam boilers, as well as for explosion in internal combustion engines of various kinds, Diesel engines, or the like.

An object of my invention is to provide an 20 efficient fuel for various uses, which fuel, although containing a comparatively heavy hydrocarbon, shall nevertheless contain such additional substance or substances as to enable the fuel to be used, alternatively or optionally, in the same manner as the familiar light hydrocarbon fuels heretofore employed 25 in internal combustion engines, or the like, said additional substances not being mere paraffin hydrocarbons.

Another object of my invention is to provide 30 a fuel or type of fuel, containing a relatively heavy hydrocarbon, together with an additional lighter combustible ingredient of such a character that it will blend effectually with the relatively heavy hydrocarbon and notably modify the properties thereof.

In one of its broader aspects, my present 35 invention may be said to aim at a wider availability, in the production of motive power, on the part of relatively heavy hydrocarbons, such as heavy distillates which may 40 be derived from crude oil and which may have a Baumé gravity of less than 40°, such wider availability resulting from the employment therewith of an ingredient or ingredients which shall contribute so notably 45 to readiness of ignition that satisfactory ignition may be obtained without raising the Baumé density of the product even to the level of ordinary kerosene, and contribute to producing an improved combustion, and in one of its more restricted aspects my present invention may be said to 50 aim at the production, from hydrocarbons that have already been deprived of their gasoline and kerosene fractions, of a prod-

uct, presumably less costly than either of the mentioned fractions, which shall at the same time rival gasoline in its suitability for use in, for example, automobile engines.

In one aspect, the present invention may be said to proceed from a recognition of progress made and to be made in the design of engines and other devices for the utilization of the energy of fuels, and, in so far as it aims at a supplemental advance in the perfecting of supposedly inferior fuels for more exacting and important uses than those to which such fuels have heretofore been put, it may be said to aim at the obviating of a shortage in one of the prime necessities of modern manufacture and commerce, fuels for automobiles engines and the like.

The fuels herein referred to being essentially mere mixtures or solutions of one or organic substance within another, it will be apparent that the sequence of operations by which they are produced may be varied, but the following may serve as typical examples.

When I begin with any ordinary mineral oil, such as a typical Pennsylvania crude oil, I may first distill off for direct use in commerce the usual quantities of lighter products including gasoline and kerosene, proceeding with such distillation preferably until substantially all the gasoline and kerosene have been distilled off and until the residuum left in the still shall have a Baumé gravity less than 40°. I may then associate with this residual material, or with a fraction distilled therefrom, and in any convenient manner, as by pouring and agitating, or by distilling directly thereinto, one or more relatively volatile combustible constituents satisfactorily miscible therewith, such as:

Alcohols (e. g. methyl, ethyl, propyl, butyl or amyl alcohol, or mixtures thereof).

Ethers (e. g. ethyl, methyl or ethyl methyl ether, or mixtures thereof).

Esters (e. g. esters made from any of the above alcohols and any organic acid, or mixtures containing such esters).

Ketones (e. g. acetone, methyl ethyl ketone, or oils or other mixtures containing such ketones).

The foregoing types of relatively volatile combustible constituents may, for convenience be generically referred to in this case or in related cases as organic compounds con-

taining an alkyl radicle and oxygen, the esters and ketones being somewhat more specifically referred to collectively as organic compounds containing a carbonyl group and an alkyl radicle.

The proportions in which the respectively volatile combustible ingredients referred to (or any analogous ingredients that may fall within the claims hereinafter presented) 10 may advantageously be incorporated with the heavier hydrocarbon or hydrocarbon mixture will, of course, depend not alone upon the exact character of the heavy hydrocarbon and upon the selection made 15 among the volatile combustible ingredients, but also upon whether it is intended to produce in one product what might be termed a "versatile" or "universal" liquid fuel capable of a great variety of uses, or whether the 20 manufacturing intent is rather to produce a fuel possessing, in the highest practicable degree, certain advantages or peculiarities adapting it to some specific use (such as use in vehicle engines, in stationary engines, in 25 injection oil engines, or in oil burners), and an extremely wide range of variations will accordingly be understood to be included within the intended scope of the claims appended hereto. The following are offered 30 merely as specific examples of compositions within the scope of my present invention, it being understood that wherever the expression "heavy oil" is employed in the said examples, this expression may refer to a petroleum distillate or residue which may consist of paraffin oils and which may be heavier than 40° Bé., and which may, for example, be as heavy as 28° Bé. By the term "petroleum distillates heavier than kerosene", I 35 mean those petroleum distillates which have densities lying above the generally-accepted upper limit of the range of kerosene densities, which, as already mentioned, lies at about 40° Bé., or about .82 absolute density. 40 The parts therein referred to are parts by volume:

#### GROUP I.

##### Example 1.

|    |                                 |    |        |
|----|---------------------------------|----|--------|
| 50 | Heavy oil                       | 75 | parts. |
|    | Alcohol (of about 95% strength) | 15 | parts. |
|    | Ether                           | 5  | parts. |
|    | Ethyl acetate                   | 5  | parts. |

##### Example 2.

|    |                                 |    |        |
|----|---------------------------------|----|--------|
| 55 | Heavy oil                       | 70 | parts. |
|    | Alcohol (of about 95% strength) | 20 | parts. |
|    | Ether                           | 4  | parts. |
|    | Ethyl acetate                   | 3  | parts. |
|    | Acetone                         | 3  | parts. |

60 It should be understood that, in any of the examples of the foregoing Group I, the alcohol may, within the scope of the present invention, be supplanted wholly or in part by 65 a corresponding quantity of one or more of

the alternative oxygen-containing volatile alkyl compounds mentioned in the same or another example.

#### GROUP II.

##### Example 3.

|               |    |        |
|---------------|----|--------|
| Heavy oil     | 80 | parts. |
| Ethyl acetate | 20 | parts. |

##### Example 4.

|           |    |        |
|-----------|----|--------|
| Heavy oil | 83 | parts. |
| Acetone   | 17 | parts. |

It should be understood that in the preparation of fuels within Group II, the quantity of acetone recommended is slightly less than the quantity of ethyl acetate recommended. Due allowance being made for this difference, acetone may be substituted for ethyl acetate in whole or in part, these mentioned volatile constituents being alike in containing the group CO, which, as hereinbefore mentioned, justifies reference to them generically, in the appended claims, as compounds containing carbonyl and alkyl.

As already mentioned, and as will be apparent from the foregoing, while I have described in detail numerous specific embodiments of my invention in "universal" liquid fuels, each of them comprising a preponderating quantity of a heavy hydrocarbon, and each of them suitable for uses as widely separated as are, on the one hand, employment (under suitable conditions of temperature and pressure and in due admixture with air or with oxygen) in explosion motors and, on the other hand, employment in direct generation of heat under steam boilers, many additional changes may be made without departing from the spirit of my invention, as indicated in the foregoing description and in the appended claims.

I claim:

1. A liquid fuel comprising a petroleum distillate heavier than kerosene and an ester of an organic acid and a mono-hydric alcohol, the heavy oil being present in the proportion of about three-quarters of the total mixture.

2. A liquid fuel comprising a petroleum distillate heavier than kerosene and an ester of an organic acid and a mono-hydric alcohol, the heavy oil and the ester being present in the proportions of about 70 to 80 parts oil and about 3 to 20 parts ester.

3. A liquid fuel comprising a petroleum distillate heavier than kerosene and an ester of an organic acid and mono-hydric alcohol, an alcohol, an ether, and a ketone, in the respective proportions of about 70 parts heavy oil, 3 parts ester, 20 parts alcohol, 4 parts ether and about 3 parts ketone.

4. A liquid fuel comprising a petroleum distillate heavier than kerosene, an ester of an organic acid and a mono-hydric alco-

- hol, and an alcohol, in the respective proportions of about 70 parts oil, about 3 parts ester and about 20 parts alcohol.
5. A liquid fuel comprising a petroleum distillate heavier than kerosene, and ethyl acetate in proportions of about 70 to 80 parts oil and 3 to 20 parts ethyl acetate.
6. A liquid fuel comprising a petroleum distillate heavier than kerosene, ethyl acetate, and an alcohol, in the proportions of about 70 parts oil, about 20 parts alcohol and about 3 parts acetate.
7. A liquid fuel comprising a petroleum distillate heavier than kerosene, ethyl acetate, and an ether, in the proportions of about 70 parts oil, about 3 parts acetate and about 4 parts ether.
8. A liquid fuel comprising a petroleum distillate heavier than kerosene, and an ester of an organic acid and a mono-hydric alcohol.
9. A liquid fuel comprising a petroleum distillate heavier than kerosene, an ester of an organic acid and mono-hydric alcohol, and an alcohol.
10. A liquid fuel comprising a petroleum distillate heavier than kerosene, an ester of an organic acid and mono-hydric alcohol, and an alcohol.
11. A liquid fuel comprising a petroleum distillate heavier than kerosene, an ester of an organic acid and mono-hydric alcohol, an alcohol, and an ether.
12. A liquid fuel comprising a petroleum distillate heavier than kerosene, an ester of an organic acid and mono-hydric alcohol, an alcohol, an ether, and a ketone.
13. A liquid fuel comprising a petroleum distillate heavier than kerosene, an ester of an organic acid and mono-hydric alcohol, and an ether.
14. A liquid fuel comprising a petroleum distillate heavier than kerosene, an ester of an organic acid and mono-hydric alcohol, and a ketone.
15. A liquid fuel comprising a petroleum distillate heavier than kerosene, an ester of an organic acid and mono-hydric alcohol, an ether, and a ketone.
- 45
- In testimony that I claim the foregoing, 50 I have hereunto set my hand this 16th day of March, 1920.

BURNELL R. TUNISON.